# EUROPEAN PATENT SPECIFICATION

(11) **EP 2 718 937 B1**
(45) Date of publication and mention of the grant of the patent: **22.07.2015**
(21) Application number: 12727084.1
(22) Date of filing: 07.06.2012
(51) Int. Cl.: H01B 1/22, H01B 1/16

(54) **THICK FILM PASTE CONTAINING BISMUTH-BASED OXIDE AND ITS USE IN THE MANUFACTURE OF SEMICONDUCTOR DEVICES**
DICKSCHICHTPASTE MIT EINEM OXID AUF WISMUTBASIS UND IHRE VERWENDUNG BEI DER HERSTELLUNG VON HALBLEITERBAUELEMENTEN
PÂTE POUR FILMS ÉPAIS CONTENANT UN OXYDE À BASE DE BISMUTH ET SON UTILISATION DANS LA FABRICATION DE DISPOSITIFS À SEMI-CONDUCTEURS

(30) Priority: 13.06.2011 US 201161496106 P
(43) Date of publication of application: 16.04.2014
(73) Proprietor: E. I. du Pont de Nemours and Company, Wilmington, DE 19898 (US)
(72) Inventor: HANG, Kenneth, Warren, Cary, NC 27519 (US); WANG, Yueli, Cary, NC 27519 (US)
(74) Representative: Hoffmann, Benjamin
(86) International application number: PCT/US2012/041325
(87) International publication number: WO 2012/173863

(56) References cited:
- EP-A1- 0 463 826
- US-A1- 2009 188 555
- US-A1- 2009 189 126

## Description

### FIELD OF THE INVENTION

The present invention is directed primarily to a thick film paste composition and thick film electrodes formed from the composition. It is further directed to a silicon semiconductor device and, in particular, it pertains to the electroconductive composition used in the formation of a thick film electrode of a solar cell. The present invention is also directed to a bismuth-based oxide that serves as a component of thick film pastes.

### TECHNICAL BACKGROUND OF THE INVENTION

The present invention can be applied to a broad range of semiconductor devices, although it is especially effective in light-receiving elements such as photodiodes and solar cells. The background of the invention is described below with reference to solar cells as a specific example of the prior art.

A conventional solar cell structure with a p-type base has a negative electrode that is typically on the front-side or sun side of the cell and a positive electrode on the back side. Radiation of an appropriate wavelength falling on a p-n junction of a semiconductor body serves as a source of external energy to generate hole-electron pairs in that body. Because of the potential difference which exists at a p-n junction, holes and electrons move across the junction in opposite directions and thereby give rise to flow of an electric current that is capable of delivering power to an external circuit. Most solar cells are in the form of a silicon wafer that has been metallized, i.e., provided with metal electrodes that are electrically conductive. Typically thick film pastes are screen printed onto substrate and fired to form the electrodes.

An example of this method of production is described below in conjunction with FIGURES 1A - 1F.

FIG. 1A shows a single crystal or multi-crystalline p-type silicon substrate 10.

In FIG. 1B, an n-type diffusion layer 20 of the reverse conductivity type is formed by the thermal diffusion of phosphorus using phosphorus oxychloride as the phosphorus source. In the absence of any particular modifications, the diffusion layer 20 is formed over the entire surface of the silicon p-type substrate 10. The depth of the diffusion layer can be varied by controlling the diffusion temperature and time, and is generally formed in a thickness range of about 0.3 to 0.5 microns. The n-type diffusion layer may have a sheet resistivity of several tens of ohms per square up to about 120 ohms per square.

After protecting the front surface of this diffusion layer with a resist or the like, as shown in FIG. 1C the diffusion layer 20 is removed from the rest of the surfaces by etching so that it remains only on the front surface. The resist is then removed using an organic solvent or the like.

Then, as shown in FIG. 1D an insulating layer 30 which also functions as an anti-reflection coating is formed on the n-type diffusion layer 20. The insulating layer is commonly silicon nitride, but can also be a SiNₓ:H film (i.e., the insulating film comprises hydrogen for passivation during subsequent firing processing), a titanium oxide film, a silicon oxide film, or a silicon oxide/titanium oxide film. A thickness of about 700 to 900 A of a silicon nitride film is suitable for a refractive index of about 1.9 to 2.0. Deposition of the insulating layer 30 can be by sputtering, chemical vapor deposition, or other methods.

Next, electrodes are formed. As shown in FIG. 1E, a silver paste 500 for the front electrode is screen printed on the silicon nitride film 30 and then dried. In addition, a back side silver or silver/aluminum paste 70, and an aluminum paste 60 are then screen printed onto the back side of the substrate and successively dried. Firing is carried out in an infrared furnace at a temperature range of approximately 750 to 850°C for a period of from several seconds to several tens of minutes.

Consequently, as shown in FIG. 1F, during firing, aluminum diffuses from the aluminum paste 60 into the silicon substrate 10 on the back side thereby forming a p+ layer 40 containing a high concentration of aluminum dopant. This layer is generally called the back surface field (BSF) layer, and helps to improve the energy conversion effciency of the solar cell.

Firing converts the dried aluminum paste 60 to an aluminum back electrode 61. The back side silver or silver/aluminum paste 70 is fired at the same time, becoming a silver or silver/aluminum back electrode, 71. During firing, the boundary between the back side aluminum and the back side silver or silver/aluminum assumes the state of an alloy, thereby achieving electrical connection. Most areas of the back electrode are occupied by the aluminum electrode 61, owing in part to the need to form a p+ layer 40. Because soldering to an aluminum electrode is impossible, the silver or silver/aluminum back electrode 71 is formed over portions of the back side as an electrode for interconnecting solar cells by means of copper ribbon or the like. In addition, the front side silver paste 500 sinters and penetrates through the silicon nitride film 30 during firing, and thereby achieves electrical contact with the n-type layer 20. This type of process is generally called "fire through." The fired electrode 501 of FIG 1F clearly shows the result of the fire through.

US 2009/189126 A1 discloses a glass frit comprising TeO2, Bi2O3 and B2O3 and other oxides like ZnO, Al2O3 and BaO. Silver, gold, copper, platinum are used as conductive materials. The glass frit is lead-free.

There is an on-going effort to provide thick film paste compositions that have reduced amounts of silver and are Pb-free while at the same time maintaining electrical performance and other relevant properties of the resulting electrodes and devices. The present invention provides a silver paste composition that simultaneously provides a Pb-free system with lower amounts of Ag while still maintaining electrical and mechanical performance.

### SUMMARY OF THE INVENTION

The present invention provides a thick film paste composition comprising:
(a) 35-55 wt% Ag;
(b) 0.5-5 wt% Pb-free bismuth-based oxide; and
(c) organic medium;
wherein the Ag and the bismuth-based oxide are dispersed in the organic medium and wherein the wt% are based on the total weight of the paste composition, the bismuth-based oxide comprising 66-78 wt% Bi₂O₃, 10-18 wt% ZnO, 5-14 wt% B₂O₃, 0.1-5 wt% Al₂O₃, 0.3-9 wt% BaO and 0-3 wt% SiO₂, based on the total weight of the bismuth-based oxide, wherein the bismuth-based oxide is Pb-free.

In one embodiment, the thick film paste composition comprises 2-5 wt % Bi-based oxide..

The invention also provides a semiconductor device, and in particular, a solar cell comprising an electrode formed from the instant paste composition, wherein the paste composition has been fired to remove the organic medium and form the electrode.

### BRIEF DESCRIPTION OF THE FIGURES

Figures 1A - 1F illustrate the fabrication of a semiconductor device. Reference numerals shown in Figure 1 are explained below.
   - 10:: p-type silicon substrate
   - 20:: n-type diffusion layer
   - 30:: silicon nitride film, titanium oxide film, or silicon oxide film
   - 40:: p+ layer (back surface field, BSF)
   - 60:: aluminum paste formed on back side
   - 61:: aluminum back side electrode (obtained by firing back side aluminum paste)
   - 70:: silver/aluminum paste formed on back side
   - 71:: silver/aluminum back side electrode (obtained by firing back side silver/aluminum paste)
   - 500:: silver paste formed on front side
   - 501:: silver front electrode (formed by firing front side silver paste)
Figures 2A-D explain the manufacturing process of one embodiment for manufacturing a solar cell using the electroconductive paste of the present invention. Reference numerals shown in Figure 2 are explained below.
   - 102: silicon substrate with diffusion layer and an anti-reflection coating
   - 104: light-receiving surface side electrode
   - 106: paste composition for Al electrode
   - 108: paste composition of the invention for tabbing electrode
   - 110: Al efectrode
   - 112: tabbing electrode

### DETAILED DESCRIPTION OF THE INVENTION

The conductive thick film paste composition of the instant invention contains a reduced amount of silver but simultaneously provides the ability to form an electrode from the paste wherein the electrode has good electrical and adhesion properties.

The conductive thick film paste composition comprises silver, a bismuth-based oxide that is Pb-free, and an organic vehicle. It is used to form screen printed electrodes and, particularly, to form tabbing electrodes on the back side on the silicon substrate of a solar cell. The paste composition comprises 35-55 wt% silver, 0.5-5 wt% bismuth-based oxide and an organic medium, wherein the Ag and the bismuth-based oxide are both dispersed in the organic medium and wherein the weight percentages are based on the total weight of the paste composition.

Each component of the thick film paste composition of the present invention is explained in detail below.

### Silver

In the present invention, the conductive phase of the paste is silver (Ag). The silver can be in the form of silver metal, alloys of silver, or mixtures thereof. Typically, in a silver powder, the silver particles are in a flake form, a spherical form, a granular form, a crystalline form, other irregular forms and mixtures thereof. The silver can be provided in a colloidal suspension. The silver can also be in the form of silver oxide (Ag₂O), silver salts such as AgCl, AgNO₃, AgOOCCH₃ (silver acetate), AgOOCF₃ (silver trifluoroacetate}, silver orthophosphate (Ag₃PO₄), or mixtures thereof. Other forms of silver compatible with the other thick-flm paste components can also be used.

In one embodiment, the thick-film paste composition comprises coated silver particles that are electrically conductive. Suitable coatings include phosphorous and surfactants. Suitable surfactants include polyethyleneoxide, polyethyleneglycol, benzotriazole, poly(ethyleneglycol)acetic acid, lauric acid, oleic acid, capric acid, myristic acid, linolic acid, stearic acid, palmitic acid, stearate salts, palmitate salts, and mixtures thereof. The salt counter-ions can be ammonium, sodium, potassium, and mixtures thereof.

The particle size of the silver is not subject to any particular limitation. In one embodiment, an average particle size is less than 10 microns; in another embodiment, the average particle size is less than 5' microns.

As a result of its cost, it is advantageous to reduce the amount of silver in the paste while maintaining the required properties of the paste and the electrode formed from the paste. In addition, the instant thick film paste enables the formation of electrodes with reduced thickness, resulting in further savings. The instant thick film paste composition comprises 35-55 wt% silver, based on the total weight of the paste composition. In one embodiment the thick film paste composition comprises 38-52 wt% silver.

### Bismuth-Based Oxide

A component of the paste composition is a lead-free bismuth-based oxide. In an embodiment, this oxide may be a glass composition, e.g., a glass frit. In a further embodiment, this oxide may be crystalline, partially crystalline, amorphous, partially amorphous, or combinations thereof. In an embodiment, the bismuth-based oxide may include more than one glass composition. In an embodiment, the bismuth-based oxide composition may include a glass composition and an additional composition, such as a crystalline composition.

The bismuth-based oxide may be prepared by mixing Bi₂O₃, ZnO, B₂O₃, Al₂O₃. BaO, SiO₂ and other oxides to be incorporated therein (or other materials that decompose into the desired oxides when heated) using techniques understood by one of ordinary skill in the art. Such preparation techniques may involve heating the mixture in air or an oxygen-containing atmosphere to form a melt, quenching the melt, and grinding, milling, and/or screening the quenched material to provide a powder with the desired particle size. Melting the mixture of bismuth oxides and the other oxides to be incorporated therein is typically conducted to a peak temperature of 800 to 1200°C. The molten mixture can be quenched, for example, on a stainless steel platen or between counter-rotating stainless steel rollers to form a platelet. The resulting platelet can be milled to form a powder. Typically, the milled powder has a d₅₀ of 0.1 to 3.0 microns. One skilled in the art of producing glass frit may employ alternative synthesis techniques such as but not limited to water quenching, sol-gel, spray pyrolysis, or others appropriate for making powder forms of glass.

The starting mixture used to make the Bi-based oxide includes 66-78 wt% Bi₂O₃, 10-18 wt% ZnO, 5-14 wt% B₂O₃, 0.1-5 wt% Al₂O₃, 0.3-9 wt% BaO and 0-3 wt% SiO₂, based on the total weight of the bismuth-based oxide. In a further embodiment, the starting mixture used to make the Bi-based oxide includes 70-75 wt% Bi₂O₃, 11-15 wt% ZnO, 7-11 wt% B₂O₃, 0.3-3.5 wt% Al₂O₃, 2-7 wt% BaO and 0.5-3 wt% SiO₂, based on the total weight of the bismuth-based oxide. In a still further embodiment, the starting mixture further includes 0.1-3 wt% of an oxide selected from the group consisting of Li₂O, SnO₂ and mixtures thereof, again based on the total weight of the starting mixture of the Bi-based oxide.

In any of the above embodiments; the Bi-based oxide may be a homogenous powder. In a further embodiment, the Bi-based oxide may be a combination of more than one powder, wherein each powder may separately be a homogenous population. The composition of the overall combination of the 2 powders is within the ranges described above. For example, the Bi-based oxide may include a combination of 2 or more different powders; separately, these powders may have different compositions, and may or may not be within the ranges described above; however, the combination of these powders may be within the ranges described above.

In any of the above embodiments, the Bi-based oxide composition may include one powder which includes a homogenous powder including some but not all of the desired elements of the Bi-based oxide composition, and a second powder, which includes one or more of the other desired elements. For example, a Bi-based oxide composition may include a first powder including Bi, Zn, B, Ba and O, and a second powder including Al, Si and O. In an aspect of this embodiment, the powders may be melted together to form a uniform composition. In a further aspect of this embodiment, the powders may be added separately to a thick film composition.

In embodiments containing Li₂O, some or all of the Li₂O may be replaced with Na₂O, K₂O, Cs₂O, or Rb₂O, resulting in a glass composition with properties similar to the compositions listed above.

Glass compositions, also termed glass frits, are described herein as including percentages of certain components. Specifically, the percentages are the percentages of the components used in the starting material that was subsequently processed as described herein to form a glass composition. Such nomenclature is conventional to one of skill in the art. In other words, the composition contains certain components, and the percentages of those components are expressed as a percentage of the corresponding oxide form. As recognized by one of ordinary skill in the art in glass chemistry, a certain portion of volatile species may be released during the process of making the glass. An example of a volatile species is oxygen. It should also be recognized that while the glass behaves as an amorphous material it will likely contain minor portions of a crystalline material.

If starting with a fired glass, one of ordinary skill in the art may calculate the percentages of starting components described herein using methods known to one of skill in the art including, but not limited to: Inductively Coupled Plasma-Emission Spectroscopy (ICPES), Inductively Coupled Plasma-Atomic Emission Spectroscopy (ICP-AES), and the like. In addition, the following exemplary techniques may be used: X-Ray Fluorescence spectroscopy (XRF); Nuclear Magnetic Resonance spectroscopy (NMR); Electron Paramagnetic Resonance spectroscopy (EPR); Mössbauer spectroscopy; electron microprobe Energy Dispersive Spectroscopy (EDS); electron microprobe Wavelength Dispersive Spectroscopy (WDS); Cathodo-Luminescence (CL).

Bi-based oxides of the invention can be prepared by mixing and blending Bi₂O₃, ZnO, B₂O₃, Al₂O₃, BaO and SiO₂ powders and, when present, Li₂O, and SnO₂ powders, and processing the mixture as described in Example 1. Examples of such bismuth-based oxide compositions A-J are shown in Table 1. The weight percentages.of the various component oxides are shown and are based on the weight of the total bismuth-based oxide composition.

**Table 1**

| | Bi₂O₃ | ZnO | B₂O₃ | Al₂O₃ | BaO | SiO₂ | Li₂O | SnO₂ |
|---|---|---|---|---|---|---|---|---|
| A | 70.73 | 14.49 | 8.80 | 0.64 | 2.79 | 2.04 | 0.50 | |
| B | 70.70 | 11.75 | 7.14 | 0.52 | 7.01 | 1.65 | 1.22 | |
| C | 73.00 | 13.00 | 9.50 | 0.50 | 3.00 | 1.00 | | |
| D | 73.00 | 13.20 | 8.10 | 0.85 | 2.25 | 2.60 | | |
| E | 70.00 | 14.50 | 7.50 | 3.00 | .3.50 | 1.50 | | |
| F | 70.00 | 14.50 | 7.50 | 3.00 | 3.20 | 1.50 | 0.30 | |
| G | 72.40 | 13.00 | 9.50 | 0.50 | 3.00 | 1.30 | 0.30 | |
| H | 73.20 | 13.50 | 8.20 | 0.60 | 2.60 | 1.90 | | |
| I | 74.00 | 15.00 | 10.00 | 0.50 | 0.50 | | | |
| J | 72.50 | 13.40 | 8.40 | 0.80 | 2.40 | 2.00 | | 0.50 |

One of ordinary skill in the art would recognize that the choice of raw materials could unintentionally include impurities that may be incorporated into the glass during processing. For example, the impurities may be present in the range of hundreds to thousands ppm.

The presence of the impurities would not alter the properties of the glass, the thick film composition, or the fired device. For example, a solar cell containing the thick-film composition may have the efficiency described herein, even if the thick-film composition includes impurities.

The content of the Bi-based oxide in the instant thick film paste composition is typically 0.5-5 wt%, based on the total weight of the thick film paste composition. In one embodiment, the Bi-based oxide content is 2-5 wt %.

### Organic Medium

The inorganic components of the thick-film paste composition are mixed with an organic medium to form viscous pastes having suitable consistency and rheology for printing. A wide variety of inert viscous materials can be used as the organic medium. The organic medium can be one in which the inorganic components are dispersible with an adequate degree of stability during manufacturing, shipping and storage of the pastes, as well as on the printing screen during the screen-printing process.

Suitable organic media have rheological properties that provide stable dispersion of solids, appropriate viscosity and thixotropy for screen printing, appropriate wettability of the substrate and the paste solids, a good drying rate, and good firing properties. The organic medium can contain thickeners, stabilizers, surfactants, and/or other common additives. One such thixotropic thickener is thixatrol. The organic medium can be a solution of polymer(s) in solvent(s). Suitable polymers include ethyl cellulose, ethylhydroxyethyl cellulose, wood rosin, mixtures of ethyl cellulose and phenolic resins, polymethacrylates of lower alcohols, and the monobutyl ether of ethylene glycol monoacetate. Suitable solvents include terpenes such as alpha- or beta-terpineol or mixtures thereof with other solvents such as kerosene, dibutylphthalate, butyl carbitol, butyl carbitol acetate, hexylene glycol and alcohols with boiling points above 150°C, and alcohol esters. Other suitable organic medium components include: bis(2-(2-butoxyethoxy)ethyl adipate, dibasic esters such as DBE, DBE-2, DBE-3, DBE-4, DBE-5, DBE-6, DBE-9, and DBE 1B, octyl epoxy tallate, isotetradecanol, and pentaerythritol ester of hydrogenated rosin. The organic medium can also comprise volatile liquids to promote rapid hardening after application of the thick-film paste composition on a substrate.

The optimal amount of organic medium in the thick-film paste composition is dependent on the method of applying the paste and the specific organic medium used. The instant thick-film paste composition contains 35 to 60 wt% of organic medium, based on the total weight of the paste composition.

If the organic medium comprises a polymer, the polymer typically comprises 8 to 15 wt% of the organic composition.

### Inorganic Additives

The Bi-based oxide used in the composition of the present invention provides adhesion. However, an inorganic adhesion promoter may be added to increase adhesion characteristics. This inorganic additive may be selected from the group consisting of Bi₂O₃, TiO₂, Al₂O₃, B₂O₃, SnO₂, Sb₂O₅, Cr₂O₃, Fe₂O₃, ZnO, CuO, Cu₂O, MnO₂, Co₂O₃, NiO, RuO₂, a metal that can generate a listed metal oxide during firing, a metal compound that can generate a listed metal oxide during firing, and mixtures thereof. The additive can help increase adhesion characteristics, without affecting electrical performance and bowing.

The average diameter of the inorganic additive is in the range of 0.5-10.0 µm, or dispersed to the molecular level when the additives are in the form of organo-metallic compounds. The amount of additive to be added to the paste composition is 0.01-5 wt%, based on the total weight of the paste composition.

In any of the above embodiments, the paste may further comprise 1-5 wt% aluminum (Al), based on the total weight of the paste composition. The Al is preferably in the powder form.

### Preparation of the Thick Film Paste Composition

In one embodiment, the thick film paste composition can be prepared by mixing Ag powder, the Bi-based oxide powder, and the organic medium and any inorganic additive in any order. In some embodiments, the inorganic materials are mixed first, and they are then added to the organic medium. In other embodiments, the Ag powder which is the major portion of the inorganics is slowly added to the organic medium. The viscosity can be adjusted, if needed, by the addition of solvents. Mixing methods that provide high shear are useful. The thick film paste contains less than 70 wt% of inorganic components, i.e., the Ag powder, the Bi-based oxide powder and any inorganic additives, based on the total weight of the paste composition. In an embodiment the thick film paste contains less than 60 wt% of inorganic components

The thick film paste composition can be deposited by screen-printing, plating, extrusion, inkjet, shaped or multiple printing, or ribbons.

In this electrode-forming process, the thick film paste composition is first dried and then heated to remove the organic medium and sinter the inorganic materials. The heating can be carried out in air or an oxygen-containing atmosphere. This step is commonly referred to as "firing." The firing temperature profile is typically set so as to enable the burnout of organic binder materials from the dried thick film paste composition, as well as any other organic materials present. In one embodiment, the firing temperature is 750 to 950°C. The firing can be conducted in a belt furnace using high transport rates, for example, 100 - 500 cm/min, with resulting hold-up times of 0.05 to 5 minutes. Multiple temperature zones, for example 3 to 11 zones, can be used to control the desired thermal profile.

An example in which a solar cell is prepared using the paste composition of the present invention is explained with reference to Figures 2A - 2D.

First, a Si substrate 102 with a diffusion layer and an anti-reflection coating is prepared. On the light-receiving front side face (surface) of the Si substrate, electrodes 104 typically mainly composed of Ag are installed as shown in Figure 2A. On the back face of the substrate, aluminum paste, for example, PV333, PV322 (commercially available from the DuPont co., Wilmington, DE), is spread by screen printing and then dried 106 as shown in Figure 2B. The paste composition of the present invention is then spread in a partially overlapped state with the dried aluminum paste and is then dried 108 as shown in Figure 2C. The drying temperature of each paste is preferably 150°C or lower. Also, the overlapped part of the aluminum paste and the paste of the invention is preferably about 0.5-2.5 mm.

Next, the substrate is fired at a temperature of 700-950°C for about 1-15 min so that the desired solar cell is obtained as shown in Figure 2D. The electrodes 112 are formed from the paste composition of the present invention wherein the composition has been fired to remove the organic medium and sinter the inorganics. The solar cell obtained has electrodes 104 on the light-receiving front side of the substrate 102, and Al electrodes 110 mainly composed of Al and electrodes 112 composed of the fired paste composition of the present invention on the back face. The electrodes 112 serve as a tabbing electrode on the back side of the solar cell.

### EXAMPLES

### Example 1

### Bismuth-Based Oxide Preparation

A bismuth-based oxide composition was prepared by mixing and blending Bi₂O₃, ZnO, B₂O₃, Al₂O₃, BaO and SiO₂ powders to result in a Bi-based oxide composition comprising 73.00 wt% Bi₂O₃, 13.00 wt % ZnO, 9.50 wt% B₂O₃, 0.5 wt% Al₂O₃, 3.00 wt% BaO, and 1.00 wt% SiO₂. The blended powder batch materials were loaded to a platinum alloy crucible then inserted into a furnace and heated at 900°C in air or O₂ for one hour to melt the mixture. The liquid melt was quenched from 900°C by removing the platinum crucible from the furnace and pouring the melt through counter rotating a stainless steel rollers gapped to 0.010 -0.020". The resulting material was coarsely crushed in a stainless steel container. The crushed material was then ball-milled in an alumina-silicate ceramic ball mill with zirconia media and water until the d₅₀ was 0.5-0.7 microns. The ball-milled material was then separated from the milling balls, wet screened and dried by hot air oven. The dried powder was run through a 200 mesh screen to provide the Bi-based oxide powder used in the thick film paste preparations described below. X-ray analysis of the powder showed a characteristic of an amorphous material. The material was characterized by Thermo-mechanical Analysis (TMA) and shows an onset of particle sintering at 320°C which transitions to fully viscous flow at 353°C. The liquidus for the composition appears to be near 511°C (between 320°C and 511 °C some crystalline phases may be transiently formed and re-dissolved in the region between sintering onset and the liquidus temperature).

### Thick Film Paste Composition Preparation

The thick film paste was prepared by mixing Ag, the Bi-based oxide powder prepared above in Example 1, organic medium, thixatrol and adhesion promoters. The Ag, the Bi-based oxide and the adhesion promoters were added to the organic medium and the thixatrol with continued stirring. Since the silver was the major portion of the solids it was added slowly to insure better wetting. The paste was then passed through a three-roll mill at a 1 mil gap several times. The degree of dispersion was measured by fine of grind (FOG) to insure that the FOG was less than or equal to 20/10.

The proportions of ingredients used in this Example were 50 wt% Ag, 2.0 wt% Bi-based oxide, 45.25 wt% organic medium, 0.75 wt% thixatrol, and 2.0 wt% inorganic adhesion promoter made up of 1.0 wt% ZnO, 0.6 wt% Bi₂O₃ and 0.4 wt% Cu.

### Test Electrodes

In order to determine the adhesion properties of electrodes formed from the instant paste composition, the paste composition was screen printed onto a silicon wafer surface in the form of an electrode. The paste was then dried and fired in a furnace. The dried thickness of the sample was 3.1 µm.

### Test Procedure-Adhesion

After firing, a solder ribbon was soldered to the fired paste. Since the current invention comprises only Pb-free Bi-based oxide, Pb-free solder was used. The Pb-free solder used was 96.5Sn/3.5Ag. Solder temperature for the Pb-free solder was in the range of 345-375°C, solder time was 5-7s. Flux used was MF200.

The soldered area was approximately 2mm x 2mm. The adhesion strength was obtained by pulling the ribbon at an angle of 90° to the surface of the cell. An assessment of the adhesion strength was assigned as low, adequate, or good, based on the assumption that an adhesion strength less than 200g is considered low; values in the range of 200g to 300g is adequate, values in the range of 300 to 400 or above is good.

Adhesion was determined for the as-prepared sample of Example 1 and the average of 18 measurements was 661 g.

### Example 2

Example 2 was carried out as described in Example 1 except that the paste was prepared using 50 wt% Ag, 3.3 wt% Bi-based oxide, 43.95 wt% organic medium, 0.75 wt% thixatrol, and 2.0 wt% inorganic adhesion promoter made up of 1.0 wt% ZnO, 0.6 wt% Bi₂O₃ and 0.4 wt% Cu. The dried thickness of the sample was 3.2 µm.

Adhesion was determined for the sample of Example 2 as described in Example 1. The average adhesion for the as-prepared sample was 451 g.

### Example 3

Example 3 was carried out as described in Example 1 except that the paste was prepared using 52 wt% Ag, 4.5 wt% Bi-based oxide, 40.75 wt% organic medium, 0.75 wt% thixatrol, and 2.0 wt% inorganic adhesion promoter made up of 1.0 wt% ZnO, 0.6 wt% Bi₂O₃ and 0.4 wt% Cu. The dried thickness of the sample was 6.5 µm.

Adhesion was determined for the sample of Example 3 as described in Example 1. The average adhesion for the as-prepared sample was 788 g.

### Example 4

Example 4 was carried out as described in Example 1 except that the paste was prepared using 55 wt% Ag, 4.5 wt% Bi-Te-O, 37.75 wt% organic medium, 0.75 wt% thixatrol, and 2.0 wt% inorganic adhesion promoter made up of 1.0 wt% ZnO, 0.6 wt% Bi₂O₃ and 0.4 wt% Cu. The dried thickness of the sample was 6.1 µm.

Adhesion was determined for the sample of Example 4 as described in Example 1. The average adhesion for the as-prepared sample was 798 g.

## Claims

1. A thick film paste composition comprising:
(a) 35-55 wt% Ag;
(b) 0.5-5 wt% Pb-free bismuth-based oxide; and
(c) an organic medium;
wherein said Ag and said bismuth-based oxide are dispersed in said organic medium and wherein said wt% are based on the total weight of said thick film paste composition, said bismuth-based oxide comprising 66-78 wt% Bi₂O₃, 10-18 wt% ZnO, 5-14 wt% B₂O₃, 0.1-5 wt% Al₂O₃, 0.3-9 wt% BaO and 0-3 wt% SiO₂, based on the total weight of said bismuth-based oxide.

2. The thick film paste composition of claim 1, said thick film paste composition comprising 2-5 wt% bismuth-based oxide, wherein said wt% are based on the total weight of said thick film paste composition.

3. The thick film paste composition of claim 1, said bismuth-based oxide comprising 70-75 wt% Bi₂O₃, 11-15 wt% ZnO, 7-11 wt% B₂O₃, 0.3-3.5 wt% Al₂O₃, 2-7 wt% BaO and 0.5-3 wt% SiO₂, based on the total weight of said bismuth-based oxide.

4. The thick film paste composition of claim 1, said bismuth-based oxide further comprising 0.1-3 wt% of an oxide selected from the group consisting of Li₂O, SnO₂ and mixtures thereof, based on the total weight of said bismuth-based oxide.

5. The thick film paste composition of claim 1, further comprising 0.01-5 wt% of an inorganic additive selected from the group consisting of Bi₂O₃, TiO₂, Al₂O₃, B₂O₃, SnO₂, Sb₂O₅, Cr₂O₃, Fe₂O₃, ZnO, CuO, Cu₂O, MnO₂, Co₂O₃, NiO, RuO₂, a metal that can generate a listed metal oxide during firing, a metal compound that can generate a listed metal oxide during firing, and mixtures thereof, wherein said wt% is based on the total weight of said thick film paste composition.

6. The thick film paste composition of claim 1, further comprising 1-5 wt% Al, wherein said wt% is based on the total weight of said thick film paste composition.

7. The thick film paste composition of claim 1, said paste composition comprising less than 70 wt% of inorganic components comprising said Ag, and said Bi-based'oxide, wherein said wt% is based on the total weight of said thick film paste composition.

8. The thick film paste composition of claim 5, said paste composition comprising less than 70 wt% of inorganic components comprising said Ag, said Bi-based oxide and any of said inorganic additives, wherein said wt% is based on the total weight of said thick film paste composition.

9. A solar cell comprising an electrode formed from the paste composition of any of claims 1-8, wherein said paste composition has been fired to remove the organic medium and form said electrode.

10. The solar cell of claim 9, wherein said electrode is a tabbing electrode on the back side of said solar cell.

## Patentansprüche

1. Dickfilmpasten-Zusammensetzung, umfassend:
(a) 35-55 Gew.-% Ag;
(b) 0,5-5 Gew.-% Pb-freies Wismut-basiertes Oxid; und
(c) ein organisches Medium;
wobei das Ag und das Wismut-basierte Oxid in dem organischen Medium dispergiert sind und wobei die Gew.-% auf das Gesamtgewicht der Dickfilmpasten-Zusammensetzung bezogen sind, wobei das Wismut-basierte Oxid 66-78 Gew.-% Bi₂O₃, 10-18 Gew.-% ZnO, 5-14 Gew.-% B₂O₃, 0,1-5 Gew.-% Al₂O₃, 0,3-9 Gew.-% BaO und 0-3 Gew.-% SiO₂, bezogen auf das Gesamtgewicht des Wismut-basierten Oxids, umfasst.

2. Dickfilmpasten-Zusammensetzung nach Anspruch 1, wobei die Dickfilmpasten-Zusammensetzung 2-5 Gew.-% Wismut-basiertes Oxid umfasst, wobei die Gew.-% auf das Gesamtgewicht der Dickfilmpasten-Zusammensetzung bezogen sind.

3. Dickfilmpasten-Zusammensetzung nach Anspruch 1, wobei das Wismut-basierte Oxid 70-75 Gew.-% Bi₂O₃, 11-15 Gew.-% ZnO, 7-11 Gew.-% B₂O₃, 0,3-3,5 Gew.-% Al₂O₃, 2-7 Gew.-% BaO und 0,5-3 Gew.-% SiO₂, bezogen auf das Gesamtgewicht des Wismut-basierten Oxids, umfasst.

4. Dickfilmpasten-Zusammensetzung nach Anspruch 1, wobei das Wismut-basierte Oxid weiterhin 0,1-3 Gew.-% eines Oxids, gewählt aus der aus Li₂O, SnO₂ und Mischungen davon bestehenden Gruppe, umfasst, bezogen auf das Gesamtgewicht des Wismut-basierten Oxids.

5. Dickfilmpasten-Zusammensetzung nach Anspruch 1, weiterhin umfassend 0,01-5 Gew.-% eines anorganischen Zusatzes, gewählt aus der Gruppe, bestehend aus Bi₂O₃, TiO₂, Al₂O₃, B₂O₃, SnO₂, Sb₂O₅, Cr₂O₃, Fe₂O₃, ZnO, CuO, Cu₂O, MnO₂, Co₂O₃, NiO, RuO₂, einem Metall, das ein aufgelistetes Metalloxid beim Brennen erzeugen kann, einer Metallverbindung, die ein aufgelistetes Metalloxid beim Brennen erzeugen kann, und Mischungen davon, wobei die Gew.-% auf das Gesamtgewicht der Dickfilmpasten-Zusammensetzung bezogen sind.

6. Dickfilmpasten-Zusammensetzung nach Anspruch 1, die weiterhin 1-5 Gew.-% Al umfasst, wobei die Gew.-% auf das Gesamtgewicht der Dickfilmpasten-Zusammensetzung bezogen sind.

7. Dickfilmpasten-Zusammensetzung nach Anspruch 1, wobei die Pastenzusammensetzung weniger als 70 Gew.-% anorganischer Komponenten, umfassend das Ag und das Bi-basierte Oxid, umfasst, wobei die Gew.-% auf das Gesamtgewicht der Dickfilmpasten-Zusammensetzung bezogen sind.

8. Dickfilmpasten-Zusammensetzung nach Anspruch 5, wobei die Pastenzusammensetzung weniger als 70 Gew.-% anorganischer Komponenten, umfassend das Ag, das Bi-basierte Oxid und beliebige der anorganischen Zusätze, umfasst, wobei die Gew.-% auf das Gesamtgewicht der Dickfilmpasten-Zusammensetzung bezogen sind.

9. Solarzelle, umfassend eine Elektrode, die aus der Pastenzusammensetzung nach einem der Ansprüche 1-8 gebildet ist, wobei die Pastenzusammensetzung gebrannt worden ist, um das organische Medium zu entfernen und die Elektrode zu bilden.

10. Solarzelle nach Anspruch 9, wobei die Elektrode eine Tabbing-Elektrode auf der Rückseite der Solarzelle ist.

## Revendications

1. Composition de pâte pour films épais comprenant :
(a) 35 à 55 % en poids d'Ag ;
(b) 0,5 à 5 % en poids d'oxyde à base de bismuth exempt de Pb ; et
(c) un milieu organique ;
dans laquelle ledit Ag et ledit oxyde à base de bismuth sont dispersés dans ledit milieu organique et dans laquelle lesdits pourcentages en poids sont basés sur le poids total de ladite composition de pâte pour films épais, ledit oxyde à base de bismuth comprenant 66 à 78 % en poids de Bi₂O₃, 10 à 18 % en poids de ZnO, 5 à 14 % en poids de B₂O₃, 0,1 à 5 % en poids d'Al₂O₃, 0,3 à 9 % en poids de BaO et 0 à 3 % en poids de SiO₂, sur la base du poids total dudit oxyde à base de bismuth.

2. Composition de pâte pour films épais selon la revendication 1, ladite composition de pâte pour films épais comprenant 2 à 5 % en poids d'oxyde à base de bismuth, lesdits pourcentages en poids étant sur la base du poids total de ladite composition de pâte pour films épais.

3. Composition de pâte pour films épais selon la revendication 1, ledit oxyde à base de bismuth comprenant 70 à 75 % en poids de Bi₂O₃, 11 à 15 % en poids de ZnO, 7 à 11 % en poids de B₂O₃, 0,3 à 3,5 % en poids d'Al₂O₃, 2 à 7 % en poids de BaO et 0,5 à 3 % en poids de SiO₂, sur la base du poids total dudit oxyde à base de bismuth.

4. Composition de pâte pour films épais selon la revendication 1, ledit oxyde à base de bismuth comprenant en outre 0,1 à 3 % en poids d'un oxyde choisi dans le groupe constitué par Li₂O, SnO₂ et des mélanges de ceux-ci, sur la base du poids total dudit oxyde à base de bismuth.

5. Composition de pâte pour films épais selon la revendication 1, comprenant en outre 0,01 à 5 % en poids d'un additif inorganique choisi dans le groupe constitué par Bi₂O₃, TiO₂, Al₂O₃, B₂O₃, SnO₂, Sb₂O₅, Cr₂O₃, Fe₂O₃, ZnO, CuO, Cu₂O, MnO₂, Co₂O₃, NiO, RuO₂, un métal susceptible de générer un oxyde de métal répertorié à la cuisson, un composé métallique susceptible de générer un oxyde de métal répertorié à la cuisson, et des mélanges de ceux-ci, ledit pourcentage en poids étant sur la base du poids total de ladite composition de pâte pour films épais.

6. Composition de pâte pour films épais selon la revendication 1, comprenant en outre 1 à 5 % en poids d'Al, ledit pourcentage en poids étant sur la base du poids total de ladite composition de pâte pour films épais.

7. Composition de pâte pour films épais selon la revendication 1, ladite composition de pâte comprenant moins de 70 % en poids de composants inorganiques comprenant ledit Ag, et ledit oxyde à base de Bi, ledit pourcentage en poids étant sur la base du poids total de ladite composition de pâte pour films épais.

8. Composition de pâte pour films épais selon la revendication 5, ladite composition de pâte comprenant moins de 70 % en poids de composants inorganiques comprenant ledit Ag, ledit oxyde à base de Bi et tout additif parmi lesdits additifs inorganiques, ledit pourcentage en poids étant sur la base du poids total de ladite composition de pâte pour films épais.

9. Cellule solaire comprenant une électrode formée à partir de la composition de pâte selon l'une quelconque des revendications 1 à 8, dans laquelle ladite composition de pâte a été cuite pour éliminer le milieu organique et former ladite électrode.

10. Cellule solaire selon la revendication 9, dans laquelle ladite électrode est une électrode de contact au dos de ladite cellule solaire.
